

1

3,379,642

## EXTRUSION LUBRICANTS

Morris L. Nielsen, Dayton, and Roger M. Niemi, Hamilton, Ohio, assignors to Monsanto Research Corporation, St. Louis, Mo., a corporation of Delaware  
No Drawing. Filed July 7, 1967, Ser. No. 651,686  
6 Claims. (Cl. 252—29)

## ABSTRACT OF THE DISCLOSURE

An improvement in the process of metal extrusion in which a composition comprising a reaction product of melamine and a phosphorus (V) acid or anhydride is used as a lubricant. A laminar lubricant such as graphite may also be present.

## BACKGROUND OF THE INVENTION

This invention relates to the extrusion of metals and alloys having melting points above 1000° C., and particularly to means of lubricating such metals and alloys in conjunction with their passage through extrusion dies. Extrusion of metals such as copper, lead, zinc or aluminum is a well-known commercial operation. Many configurations of shapes and tubing have been made available as this technology has advanced over other methods of metalworking including casting, machining, forging, rolling, etc. Certain other metals or alloys having higher melting points, especially above 1000° C., have been less amenable to extrusion so that for them this method has been slow in developing. Such metals as steel, molybdenum, tantalum, tungsten, and superalloys require very high temperatures and pressures for extrusion and as a consequence the extruding die is subjected to considerable friction. Not only does this friction increase the amount of energy necessary to effect the extrusion, but it shortens the operating life of the die through erosion and wear. Equally important, it often results in a poorly extruded metal piece having a rough surface with scratches, pits, cracks, laps, tears and gouges. Many attempts to solve this problem have been made in the past, principally through extrusion aids or lubricating materials such as glass or graphite. In U.S. Patent 2,538,917 issued Jan. 23, 1951, to J. Sejournet et al. and in U.S. Patent 3,181,324 issued May 4, 1965, to D. Labino, various forms of glass are disclosed as extrusion lubricants. In U.S. Patent 2,757,138 issued July 31, 1965, to A. Clatot et al., graphite is shown in combination with a combustible organic substance such as sawdust and a higher metal oxide.

These various methods do not yield entirely satisfactory results. The glass may not be sufficiently softened in the short contact time that it is exposed to the hot metal, so that there may result occlusions of glass in the metal, or surface defects due to uneven lubrication and excessive wear of the die. When greases are used, the contact of hot metal with organic substances may lead to undesired carbides and surface hardening by carburization.

When graphite is used alone, extrusion is usually unsatisfactory, due to failure of the solid non-fusible graphite to flow and replenish the film of lubricant between the die and workpiece. Graphite alone suffers from the further disadvantage that it has high thermal conductivity which hastens the transfer of heat from the hot billet to the cooler die. This results in two undesirable effects: the workpiece is cooled and the die is heated.

Our present invention overcomes these and other problems.

## SUMMARY

This invention relates to an improvement in the method of extruding a metal workpiece, wherein the improvement

2

comprises applying to the surface of the workpiece a composition comprising a reaction product of melamine and a phosphorus compound selected from the class consisting of a phosphorus (V) acid and phosphorus pentoxide. The composition may also include a laminar lubricant selected from the class consisting of graphite, molybdenum disulfide, boron nitride and metal-free phthalocyanine.

The melamine phosphates prepared from melamine and various phosphorus acids, e.g. ortho-, pyro-, or metaphosphoric acid are well-known compounds. Thus, there are melamine orthophosphate,  $C_3H_6N_6 \cdot H_3PO_4$ ; melamine pyrophosphate,  $(C_3H_6N_6)_2 \cdot H_4P_2O_7$ ; melamine metaphosphate,  $C_3H_6N_6 \cdot HPO_3$ ; etc., as reported in Chemical Abstracts 42, 7781h.

By heating melamine with phosphorus pentoxide in a ratio of 2 to 4 moles of melamine to one mole of phosphorus pentoxide at 300–500° C., there is obtained a product disclosed in U.S. Patent 2,544,706 issued Mar. 13, 1951, to J. E. Malowan. We have found that these materials soften or melt at high temperature, often with decomposition, and are transformed to a viscous, fluid or partly fluid state. For example, the melamine- $P_2O_5$  composition becomes soft and tacky about 900–1000° C.

It is an object of the invention to provide a lubricant for metalworking. It is a further object to provide a lubricant for the extrusion of metals having melting points above 1000° C. It is still a further object to provide an improvement in the process of extruding metals in which a composition comprising a reaction product of melamine and a phosphorus (V) acid or anhydride is used as a lubricant.

## DESCRIPTION OF THE PREFERRED EMBODIMENTS

In the extrusion of metals having high melting points, e.g. above 1000° C., it is common practice to employ a 1500 to 2500 ton horizontal extrusion press, see for example, "Extrusion of Steel," by D. A. Edgecombe, Journal of Metals, vol. 13, page 211, 1961. The die may yield simple or complex shapes, e.g. rods, channels, etc., or may in conjunction with a mandrel yield tubing. The die may be made of a hardened tool steel, and may be coated, e.g. with  $Al_2O_3$  or  $ZrO_2$ .

In operation, the billet of metal to be extruded is heated to the extruding temperature, which varies with the metal but may be in the range 1100–2000° C. The die is generally preheated to 450–550° C., to prevent chilling the workpiece. The die lubricant is inserted and then the hot billet. The ram then moves forward at a speed of 5–6 inches/sec. and the workpiece assumes a cross-section corresponding to that of the die. In the present invention, the improvement lies in the die lubricant. The following examples illustrate certain specific embodiments of the present invention.

## Example 1

Typical formulations which we have found useful as extrusion lubricants are shown in Table 1. The melamine reaction products may be used alone or in combination with laminar lubricants such as graphite. The compositions used in the present invention are prepared by first comminuting or crushing the individual components to a finely divided state, e.g. passing a 20 mesh sieve, then thoroughly mixing the components in the desired proportions. The compositions may be used in a powdered form, e.g. by scooping into a mold having a die located at one end, thereafter ramming the heated billet in contact with the powder and thence through the die; or may be used more efficiently by molding the composition first in a pellet or disc shape which is then positioned across the die opening so that the billet is rammed directly against

it and thence through the die. Other methods of applying the composition to either the die or the workpiece may be employed, with the objective of interposing the composition between the surface of the die and the workpiece so that the composition serves to lubricate the die while the metal is being extruded. In the preparation of pellets or shaped forms, binders such as sodium silicates, animal

trusion press which permitted a pressure loading of up to 184,000 p.s.i. on the billet. Billets were machined to about 3 inches in diameter. Dies were prepared from H-21 tool steel and yielded  $\frac{1}{2}$  inch rounds. Entrance to the die had a  $120^\circ$  included angle cone.

Lubricant was introduced into the extrusion chamber as a compressed disc about 3 inches in diameter by  $\frac{1}{2}$

TABLE 1.—TYPICAL FORMULATIONS USEFUL AS EXTRUSION LUBRICANTS

| Formulations, Components                                                         | Composition, Weight percent |      |      |      |      |    |
|----------------------------------------------------------------------------------|-----------------------------|------|------|------|------|----|
|                                                                                  | A                           | B    | C    | D    | E    | F  |
| Melamine orthophosphate (1:1).....                                               | 100                         | 67   | 100  | 67   | 50   | 33 |
| Melamine-P <sub>2</sub> O <sub>5</sub> composition of U.S. Patent 2,544,706..... |                             |      |      |      |      |    |
| Graphite.....                                                                    | 33                          | 33   | 33   | 50   | 67   |    |
| Coefficient of Friction at 1,100° C.....                                         | 0.1                         | 0.02 | 0.12 | 0.02 | 0.02 |    |

or vegetable glues, casein resins, polyvinyl chloride, polyvinyl acetate, polyurethanes, epoxy cements, etc., are useful for bonding the pressed composition into a suitably strong form. Sufficient binder for this purpose, usually not over 5% by weight of the total composition, may be mixed with the composition without adversely affecting its lubricating properties. Likewise, mold release agents such as stearic acid may be present, usually to the extent of not over 5% by weight.

Not only are the melamine reaction products useful lubricants per se, but by virtue of their softening and melting characteristics they may be used with and do enhance the usefulness of laminar lubricants. While we do not have a complete understanding of the mechanism by which these desirable results are achieved, we postulate that the melamine reaction products act as a matrix or dispersion medium for the laminar lubricants. We have found that intimate mixtures of the melamine-P<sub>2</sub>O<sub>5</sub> composition and graphite become pasty at about 900–1000° C., and we therefore presume that under the extrusion conditions this combination flows and replenishes the lubricating film between the metal surfaces. In this way the combination surprisingly produces a superior result to that obtained with either component alone. For the purposes of this invention the laminar lubricant may be present to the extent of 90% by weight of the composition; however, the preferred range is up to a maximum of 70% by weight of the composition.

#### Example 2

The coefficient of friction for these lubricants was determined in a TRW test machine as follows. A rotating member heated to about 450° C., and a stationary member heated to 1100° C., were held against each other under about 5000 p.s.i. pressure. The lubricant was applied between these members and the deceleration of the rotating member measured. The rotating member consisted of H-21 tool steel simulating a steel die; the stationary member was molybdenum-0.5% titanium. The preheated steel piece was inserted in a cylindrical cavity in the center of a rotating flywheel; the lubricant was applied; and the preheated stationary member was dropped in on top of the lubricated steel piece. The motor drive was removed from the flywheel and pressure was immediately applied to the exposed end of the stationary member. The angular velocity of the flywheel was recorded until it stopped. A plot of the angular velocity against time gave substantially a straight line whose slope was proportional to the coefficient of friction. The coefficients of friction obtained for old, established materials were acceptably close to values reported in the published literature.

Data for useful compositions of the present invention are shown in Table 1.

#### Example 3

Extrusions were performed on a 700 ton horizontal ex-

inch thick and pushed against the face of the die.

20 Billets of 4340 steel were heated to about 1150° C., in an inert atmosphere induction furnace and were transferred to the extrusion press.

The results of extrusions with two compositions as lubricants are shown in Table 2.

TABLE 2.—EXTRUSION OF 4340 STEEL USING EXTRUSION LUBRICANTS

|    | Composition From Table 1                                | Conditions, Ram Speed (in./sec.) | Results, Extruded Surface |
|----|---------------------------------------------------------|----------------------------------|---------------------------|
| 30 | B—Melamine phosphate+graphite.....                      | 5.5                              | Fair                      |
|    | D—Melamine-P <sub>2</sub> O <sub>5</sub> +graphite..... | 5.0                              | Fair                      |
|    | Graphite alone.....                                     | 5.0                              | Poor                      |

It is to be understood that although the invention has been described with specific reference to particular embodiments thereof, it is not to be so limited since changes and alterations therein may be made which are within the full intended scope of this invention as defined by the appended claims.

What we claim is:

- 40 1. In a method of extruding a metal workpiece through a die, an improvement which comprises applying to the surface of the die and the workpiece a composition comprising a reaction product of melamine and a phosphorus compound selected from the class consisting of a phosphorus (V) acid formed at about the temperature of 0°–300° C. and phosphorus pentoxide formed at about the temperature of 300°–500° C.
- 45 2. The method of claim 1 in which the reaction product is melamine orthophosphate.
- 50 3. The method of claim 1 in which the reaction product obtained by heating 2 to 4 moles of melamine with one mole of phosphorus pentoxide at 300 to 500° C.
- 55 4. The method of claim 1 in which the composition includes a laminar lubricant selected from the class consisting of graphite, molybdenum disulfide, boron nitride, and metal-free phthalocyanine.
- 60 5. The method of claim 4 in which the reaction product is melamine orthophosphate and the laminar lubricant is graphite, the graphite being present in the range of 2 to 70% by weight of the composition.
- 65 6. The method of claim 4 in which the reaction product is obtained by heating 2 to 4 moles of melamine with one mole of phosphorus pentoxide at 300 to 500° C., and the laminar lubricant is graphite, the graphite being present in the range of 2 to 70% by weight of the composition.

#### References Cited

##### UNITED STATES PATENTS

- 70 2,544,706 3/1951 Malowan ----- 260—249.6  
 3,213,024 10/1965 Blake et al. ----- 252—25  
 3,265,617 8/1966 Allen ----- 252—25

DANIEL E. WYMAN, Primary Examiner.

75 I. VAUGHN, Assistant Examiner.